

## UNITED STATES PATENT OFFICE

2,676,937

## AQUEOUS TEXTILE FINISHING COMPOSITION CONTAINING METHYLENE HIGHER FATTY ACID DIAMIDES

Frank M. Schofield, Woodstown, N. J., assignor to E. I. du Pont de Nemours and Company, Wilmington, Del., a corporation of Delaware

No Drawing. Application January 9, 1952,  
Serial No. 265,715

4 Claims. (Cl. 260—29.4)

1

This invention relates to textile finishing compositions and particularly to compositions which impart water-repellency and dimensional stability to fabrics which are treated therewith.

There has been a demand in the textile trade recently for cellulosic fabrics which are water-repellent, crease-resistant, dimensionally stable and which have a firm hand. Water-repellency may be obtained by the use of a number of known hydrophobic materials, one of which is methylenedistearamide. A variety of resins may be applied in order to secure the desired degree of dimensional stability. The various water-repellent agents are insoluble in water and must be applied either from non-aqueous solutions or from aqueous dispersions. The use of aqueous media is preferable from the standpoint of economy and convenience, but is often not possible because of the difficulty in preparing stable aqueous dispersions of the water-repellent agents.

It is an object of this invention to provide new compositions in the form of stable aqueous dispersions which are inexpensive and easy to apply to textile fabrics, and which produce durable water-repellency and dimensional stability in the fabric. A further object is to provide a process by which such stable aqueous dispersions are prepared. Further objects will appear from the detailed description which follows.

The compositions of this invention consist of aqueous dispersions of methylene fatty acid diamides, polyvinyl alcohol and preferably a water-soluble lower alkyl ether of a methylol melamine resin. According to the process of this invention, these compositions are prepared by: (1) heating together under vigorous agitation (a) a fatty acid amide mixture which melts between 90 to 100° C. and in which the total content of stearamide and palmitamide exceeds 80% by weight, (b) water, (c) a molecular excess of formaldehyde, and (d) from 2 to 3% by weight of a water-soluble long-chain alcohol sulfate containing from 12 to 18 carbon atoms, based on the weight of fatty acid amides, the said heating step being conducted for at least thirty minutes at a temperature between the melting point of the amide mixture and 100° C.; (2) cooling to a temperature below 80° C., adjusting the pH to below 4 and agitating for at least one hour at 75 to 85° C.; (3) filtering off the methylene fatty acid diamides and washing out the excess formaldehyde from the filter cake; (4) mixing the filter cake with from 10 to 30% polyvinyl alcohol in aqueous solution and with from 2 to 5% of a water-soluble long-chain alcohol sulfate containing from 12 to 18 carbon

2

atoms, the percentages in each case being based on the dry weight of methylene fatty acid diamides in the filter cake; and (5) mixing the resulting composition with from 0.4 to 7 parts by weight of a water-soluble lower alkyl ether of a methylol melamine resin per part of methylene fatty acid diamides.

The fatty acid amide mixture which is employed as a starting material is preferably the mixture which is sold as "technical stearamide." This product contains small amounts of free stearic acid and of stearonitrile, up to about 10%, from 50 to 95% stearamide and the balance palmitamide. Amide mixtures containing large amounts of the amides of acids having shorter chains do not provide a sufficient amount of water-repellency to be useful in this connection. Such materials may be present so long as more than 80% of the amide mixture consists of stearamide, palmitamide or a mixture thereof. In order to emulsify the fatty acid amide properly with water, it is necessary that the melting point of the amide mixture be less than 100° C. in water. Although pure stearamide is reported to melt at 109° C. and pure palmitamide at 106-107° C., the technical grade stearamide melts at about 93-98° C. in water.

A molecular excess of formaldehyde must be employed in order to obtain substantially complete reaction of the fatty acid amide. This excess must be at least 10% over the theoretical to replace formaldehyde which is lost by volatilization. It is ordinarily suitable to use a 25 to 40% excess of formaldehyde over the theoretical requirement. A much larger excess does no harm to the product but produces no corresponding advantage.

The amount of water present during formation of the dispersion is not critical so long as enough is added to give a stirrable slurry. A convenient amount is from 3 to 5 parts of water per part of fatty acid amide.

Any commercially available water-soluble long-chain alcohol sulfate can be used during the step of dispersing the amide. Particularly useful are the sodium or triethanolamine salts of the sulfates of the long-chain alcohols obtained by reduction of naturally occurring oils such as coconut oil and sperm oil. Other surface-active agents such as aromatic and aliphatic sulfonates, the sodium salts of sulfated, unsaturated long-chain esters such as the monosodium salt of sulfated methyl oleate, a betaine, and a condensate of an alkylphenol with ethylene oxide are effective in the formation of the initial dispersion.

The final composition containing the methylene fatty acid diamide, polyvinyl alcohol and resin is, however, substantially inferior when made with one of these agents as compared with the composition made with a long-chain alcohol sulfate. The preferred amount of the surface-active agent is from 2 to 3%, based on the weight of the fatty acid amide present.

During the initial heating step, some reaction occurs between the fatty acid amides and the formaldehyde, but the reaction does not proceed to completion. It is not necessary to control the pH during this period. Depending on the formic acid content of the formaldehyde, the pH at this stage is ordinarily neutral or very slightly acid.

During the second step of the process, in which the mixture is agitated at a pH below 4 at 75 to 85° C., methylol amides formed in the first step are converted to the corresponding diamides. Operation in this temperature range and for at least one hour is necessary in order to obtain satisfactory control of the physical form of the product and to secure complete reaction. Any strong acid may be used to acidify the dispersion to a pH below 4.

Vigorous agitation of the mixture is essential during the steps of forming the methylene diamide in order that the particle size of the product shall be suitably small. The dispersion obtained by this process contains the methylene diamide in the form of particles which range from about 0.5 to 5 microns.

The dispersion is dewatered by filtration or by any equivalent operation and the filter cake is then washed with water to remove any remaining excess formaldehyde. The filter cake ordinarily contains about 40 to 50% solids.

The filter cake is then mixed with polyvinyl alcohol and with a surface-active agent consisting of a water-soluble long-chain alcohol sulfate containing from 12 to 18 carbon atoms. There is added from 10 to 30% polyvinyl alcohol, based on the dry weight of methylene fatty acid diamides in the filter cake, the preferred amount being from 10 to 20%. The polyvinyl alcohol can be in the form of a commercial partially saponified polyvinyl ester. Polyvinyl acetate which is from 80 to 95% saponified is particularly suitable. The polyvinyl alcohol is added in the form of an aqueous solution.

There is added from 2 to 5% and preferably from 4 to 5% of the long-chain alcohol sulfate, based on the dry weight of methylene fatty acid diamides. Higher amounts of the surface-active agent seriously interfere with the water repellent properties of the final product. As in the initial dispersion step, any commercially available water-soluble long-chain alcohol sulfate, such as the sodium or triethanolamine salts of the sulfates of the long-chain alcohols obtained by reduction of coconut oil or sperm oil, may be used.

The filter cake containing the methylene diamides is mixed with the polyvinyl alcohol and the long-chain alcohol sulfate in any efficient mixer or colloid mill. The resulting mixture is useful directly as a textile finishing composition, producing water-repellent effects when applied to and heated on the fabrics. The effects are not as durable as when resins are also present, nor does the mixture of methylene diamide and polyvinyl alcohol produce any significant degree of dimensional stability. These mixtures are stable dispersions which may be stored or transported without adverse effect, and which may subsequently be mixed with the resin described here-

in to form the preferred compositions of this invention.

The water-soluble lower alkyl ether of a methylol melamine resin, such as a methylated methylol melamine, is most conveniently incorporated with the dispersion of methylene diamide and polyvinyl alcohol by adding the resin in aqueous solution, followed by intimate mixing. It is sometimes convenient to incorporate the resin immediately prior to application of the mixture to the fabric, although stable mixtures may be prepared in advance and shipped or stored in this state. The amount of resin to be added depends upon the nature of the fabric and of the resin and on the degree of stiffness and dimensional stability which is desired. Ordinarily at least 1 part of resin per part of methylene diamide is used, but as little as 0.4 part of resin may be used successfully. Below this amount of resin, the durability of the water-repellent effect is inferior. Amounts of resin up to about 7 parts per part of methylene diamide can be used, but at this point the compositions become undesirably expensive and water-repellency begins to decrease.

The preparation of the compositions of this invention is illustrated by the following example:

*Example 1*

A mixture of 867 parts of water, 217 parts of technical stearamide, 87 parts of 37% formaldehyde and 5 parts of a sodium alcohol sulfate derived from a mixture of alcohols containing from 10 to 16 carbon atoms, predominantly 12 and 14 carbon atoms, is heated to 96° C. with slow agitation to avoid excessive foaming. This mixture is then agitated efficiently for one hour at 96-99° C., and cooled to 75-76° C. during about thirty minutes. Then 15.5 parts of 31% hydrochloric acid are added, and the temperature rises to about 30° C., where it is held for one hour with fast, efficient agitation. The mixture gives a deep-blue color with Congo red during this period.

After addition of 200 parts of water, the charge is filtered and the cake is washed acid-free with water. The filter cake amounts to about 550 parts, containing 40% solids. The resulting methylene diamide has a melting point of 135-137° C.

The methylene diamide press cake is charged into a 40-50° C. solution containing 440 parts of 10% polyvinyl alcohol solution in water (86-89% saponified polyvinyl acetate), 50 parts of the same commercial long-chain alcohol sodium sulfate of about 20% active ingredient used in the first step, and 10 additional parts of water. The charge is made just alkaline to brilliant yellow paper (pH=7-8) by the addition of 30% sodium hydroxide solution and is agitated at 30-40° C. until it becomes a smooth, apparently homogeneous paste. It is then passed through an efficient mechanical mixer to complete the mixing.

The resulting dispersion, amounting to about 1000 parts, with a methylene diamide content of about 200 parts, is mixed with 1400 parts of a commercial methylated methylol melamine. When the resulting dispersion is diluted, mixed with ammonium acid phosphate and padded onto viscose rayon and the fabric is dried and heated for three minutes at 325-375° C., the resulting fabric possesses a high degree of water-repellency coupled with satisfactory dimensional stability and a firm hand.

Similar results are obtained when only 200

parts of methylated methylol melamine are used instead of 1400 parts.

The compositions of this invention are prepared for application to the fabric simply by mixing them into water with a small amount of any conventional mildly or potentially acidic catalyst for curing the resin. Examples of suitable catalysts include tartaric acid, the ammonium acid phosphates, zinc nitrate and the like. The aqueous dispersion is then applied to the fabric by padding or by any other convenient method. The fabric is dried and baked to cure the resin. A suitable baking period is about 3 minutes at 325 to 375° F. Generally an application of the composition sufficient to give about 1.5 to 3% of the methylene diamide on the fabric is required to obtain optimum results. The treated fabric displays excellent water-repellency, crease-resistance and dimensional stability. The hand of the fabric is improved by becoming firmer and more resilient. These effects are quite durable and survive washing and dry-cleaning of the fabric. The resin content of the composition serves not only to contribute crease-resistance and dimensional stability but also to bind the methylene diamide to the fabric so as to give a more durable water-repellent effect.

An important advantage of these compositions is that they are quite stable without close control of the pH. This is not true of many other water-repellent compositions, as for example dispersions in soap solution, which are extremely sensitive to changes in pH.

I claim:

1. A process of preparing a textile finishing composition which comprises: (1) heating together under vigorous agitation (a) a fatty acid amide mixture which melts between 90 and 100° C. in water and in which the total content of stearamide and palmitamide exceeds 80% by weight, (b) water, (c) a molecular excess of formaldehyde, and (d) from 2 to 3% by weight of a water-soluble long-chain alcohol sulfate containing from 12 to 18 carbon atoms, based on the weight of fatty acid amides, the said heating step being conducted for at least thirty minutes at a temperature between the melting point of the amide mixture and 100° C.; (2) cooling to a temperature below 80° C., adjusting the pH to below 4 and agitating for at least one hour at 75 50

to 85° C.; (3) filtering off the methylene fatty acid diamides and washing out the excess formaldehyde from the filter cake; and (4) mixing the filter cake with from 10 to 30% polyvinyl alcohol in aqueous solution and with from 2 to 5% of a water-soluble long-chain alcohol sulfate containing from 12 to 18 carbon atoms, the percentages in each case being based on the dry weight of methylene fatty acid diamides in the filter cake.

5 2. A textile finishing composition prepared by the process of claim 1.

15 3. A process of preparing a textile finishing composition which comprises: (1) heating together under vigorous agitation (a) a fatty acid amide mixture which melts between 90 and 100° C. in water and in which the total content of stearamide and palmitamide exceeds 80% by weight, (b) water, (c) a molecular excess of formaldehyde, and (d) from 2 to 3% by weight of a water-soluble long-chain alcohol sulfate containing from 12 to 18 carbon atoms, based on the weight of fatty acid amides, the said heating step being conducted for at least thirty minutes at a temperature between the melting point of the amide mixture and 100° C.; (2) cooling to a temperature below 80° C., adjusting the pH to below 4 and agitating for at least one hour at 75 to 85° C.; (3) filtering off the methylene fatty acid diamides and washing out the excess formaldehyde from the filter cake; (4) mixing the filter cake with from 10 to 30% polyvinyl alcohol in aqueous solution and with from 2 to 5% of a water-soluble long-chain alcohol sulfate containing from 12 to 18 carbon atoms, the percentages in each case being based on the dry weight of methylene fatty acid diamides in the filter cake; and (5) mixing the resulting composition with from 0.4 to 7 parts by weight of a water-soluble lower alkyl ether of a methylol melamine resin per part of methylene fatty acid diamides.

20 30 35 40 45 4. A textile finishing composition prepared by the process of claim 3.

References Cited in the file of this patent

UNITED STATES PATENTS

| Number    | Name        | Date          |
|-----------|-------------|---------------|
| 2,365,813 | Gluesenkamp | Dec. 26, 1944 |
| 2,423,428 | Pollard     | July 1, 1947  |
| 2,537,667 | Harris      | Jan. 9, 1951  |